

## UNITED STATES PATENT OFFICE

2,241,497

## WAX COMPOSITION

Jones I. Wasson, Union, and James Prophet, Jr., Cranford, N. J., assignors to Standard Oil Development Company, a corporation of Delaware

No Drawing. Application November 13, 1939,  
Serial No. 304,119

4 Claims. (Cl. 23—250)

The present invention relates to improved wax compositions. The invention is particularly concerned with the production of petroleum wax compositions of improved stability which are substantially colorless and which possess no objectionable taste or odor. The improved wax compositions of the present invention comprise a petroleum wax and a small amount of tertiary butyl ether of ortho tertiary butyl para cresol.

It is known in the art to use various inhibiting agents and the like in order to prevent the oxidation and decomposition of particular products. For example, it is known to employ various oxidation inhibitors in order to preserve the quality of high grade lubricating oils. It is also known that to some extent the effectiveness of an oxidation inhibitor when employed in one base medium may be predicted from the results secured when the oxidation inhibitor is employed in another base medium. However, the inhibition of certain products against oxidation and decomposition presents problems which cannot be solved simply by employing an oxidation inhibitor which has been found to be satisfactory when used as an oxidation inhibitor for another substance. Thus, for example, materials suitable as oxidation inhibitors for lubricating oils and the like, in general, could not be employed as oxidation inhibitors for medicinal oils and highly refined petroleum waxes. The inhibition of highly refined petroleum waxes against oxidation presents special difficulties. It is very desirable that the inhibited wax be colorless, that it be color stable, and that it be tasteless and odorless, as well as stable against oxidation. This is necessary since these waxes are oftentimes used for the production and preservation of foods and other commodities for human consumption. As a result of these requirements, very few materials are satisfactory for use as wax inhibitors.

We have now found a substance which is particularly desirable and effective for inhibiting petroleum waxes against oxidation. The inhibitor of the present invention is very effective in the prevention of oxidation of the petroleum waxes and, moreover, is particularly desirable in that it will not impair the quality of the wax.

Our inhibitor is color stable and will not impart any color, taste or odor to the inhibited highly refined wax. This inhibitor is tertiary butyl ether of ortho tertiary butyl para cresol and has the following structural formula:



This material is satisfactory for inhibiting any wax composition. It is, however, particularly effective for the production of highly refined waxes which are entirely stable and will not decompose in time or in the presence of heat. Although the inhibitor may be used to inhibit waxes having melting points in the range from about 100° F. and higher as determined by the A. S. T. M. method, it is particularly effective in the production of highly refined petroleum waxes having melting points in the range above about 120° F., preferably those having melting points in the range above about 140° F.

The quantity of the inhibitor used will vary widely, depending upon the character of the wax and the service conditions to which it will be subjected. In general, it has been found that the concentration of the inhibitor should be in the range from about 0.01% to 1.0%. It is preferred that the concentration be in the range from about 0.02% to 0.05%.

In order to more fully illustrate the invention, the following example is given which should not be construed as limiting the same in any manner whatsoever:

## EXAMPLE

Small amounts of tertiary butyl ether of ortho tertiary butyl para cresol were added to waxes and the resulting blends tested in order to determine the stability of the same. The results of these operations were as follows:

122° F. A. S. T. M. melting point wax heated for 16 hrs. at 150° C. in the presence of copper catalyst

| Per cent ether used | Initial Saybolt color | Color after oxidation test                        |
|---------------------|-----------------------|---------------------------------------------------|
| None                | +25                   | 16 1/2 Robinson color (not less than 15 Saybolt). |
| 0.01                | +25                   | 17 Robinson color (not less than 15 Saybolt).     |
| 0.02                | +25                   | +19 Saybolt.                                      |
| 0.03                | +25                   | +19 Saybolt.                                      |
| 0.05                | +25                   | +21 Saybolt.                                      |

It will be noted that 0.02% or more of the inhibitor produced a marked stabilization of the wax.

The process of the present invention is not to be limited by any theory or mode of operation, but only in and by the following claims.

We claim:

1. Improved wax composition comprising a

petroleum wax and a small amount of tertiary butyl ether of ortho tertiary butyl para cresol.

2. A wax composition in accordance with claim 1 in which the amount of tertiary butyl ether of ortho tertiary butyl para cresol is in the range from 0.02% to 0.05%.

3. A wax composition comprising a petroleum wax having a melting point above about 120° F. and from 0.01% to 1% of tertiary butyl ether of ortho tertiary butyl para cresol.

4. A wax composition characterized by being colorless, odorless, and tasteless and further characterized by being stable against oxidation and color degradation comprising a highly refined petroleum wax having a melting point in the range above about 120° F. and from 0.02% to 0.05% of tertiary butyl ether of ortho tertiary butyl para cresol.

20

JONES I. WASSON,  
JAMES PROPHET, JR.